

1

3,502,514

## METHOD OF PROCESSING STEEL

Raymond A. Grange, Washington Township, Westmoreland, Pa., assignor to United States Steel Corporation, a corporation of Delaware  
No Drawing. Filed Jan. 30, 1968, Ser. No. 701,554  
Int. Cl. C21d 7/02, 1/00

U.S. Cl. 148—12.4

8 Claims

### ABSTRACT OF THE DISCLOSURE

A method of processing carbon and low-alloy steels to develop a fibrous martensite-ferrite mixture including the steps of cold reducing steel which is preferably in the hot-rolled or heat-treated condition to at least a 50% smaller cross sectional area than initially to lengthen same, and then heating to a critical temperature ( $T_x$ ) which is determined for the steel by a specified equation and thereafter quenching to transform austenite fibers to martensite.

This invention relates to a process for strengthening hypoeutectoid steels. More particularly, the invention involves a method of processing hypoeutectoid steels to develop a fibrous martensite-ferrite mixture in carbon and low-alloy steels.

Processing condition for producing microstructures comprised of martensitic particles imbedded in a matrix of ferrite are usually avoided because such metallurgical structures have been thought of as having inferior mechanical properties. As a result, with very few exceptions carbon and low-alloy steel products are produced by processes which develop microstructures comprising carbide particles in ferrite. Recently, it has been determined that if martensite particles are sufficiently small and all elongated in the same direction, the resulting fibrous martensite-ferrite mixture may have useful properties. In fact, it has been found that such a metallurgical structure has a unique and useful combination of mechanical properties and the present invention is directed to a particularly effective method of processing steel to develop a fibrous martensite-ferrite mixture in a variety of carbon and low-alloy steels.

The process in accordance with the invention involves treating a semi-finished steel of larger cross section than the product and the process itself includes the steps of cold reducing the cross section at least 50% to desired dimensions by some cold deformation process, reheating to a particular closely controlled temperature and quenching. Initially the steel may be in a hot-rolled condition or it may have been heat treated to enhance ductility. Cold deformation may be accomplished by any means which reduces the cross section (i.e. cross sectional area) and hence lengthens the material. Examples of such cold deformation techniques include rolling, drawing, extrusion and swaging. In the second step which may follow the cold deformation in an uninterrupted sequence or may be performed later as a separate treatment, the steel is reheated to a controlled temperature within the critical range of the steel. This temperature ( $T_x$ ) is very important and varies with the chemical composition of the steel being processed. However,  $T_x$  can be calculated from the chemical composition of the steel by the following equation:

$$T_x (\text{°F.}) = 1385 - (25 \times \% \text{ Mn}) + (40 \times \% \text{ Si}) - 26 \times \% \text{ Ni} + (42 \times \% \text{ Cr})$$

Other elements may be present in the steel but are not considered in the equation because they do not significantly affect the reheat temperature in the steels with which the invention is concerned.

2

In accordance with the invention, steel which has been cold worked as described above is desirably heated to as close to the  $T_x$  temperature as possible and a reheat temperature within  $\pm 20^\circ \text{ F.}$  of  $T_x$  will usually be satisfactory. It is not necessary to hold at the  $T_x$  longer than required for the steel to reach  $T_x \pm 20^\circ \text{ F.}$  throughout. Although considerable leeway in heating time is permissible, prolonged times beyond 10 minutes are undesirable. Any method of heating may be used which permits the degree of the maximum reheat temperature throughout the steel within the specified  $T_x \pm 20^\circ \text{ F.}$  range. Preferred methods of heating include electrical induction or resistance heating or immersion in lead or salt baths. After reheating, the steel is quenched (preferably with water) to room temperature.

A consideration of the microstructural changes in the steel indicates the reason for processing the steel as described above in accordance with the invention. The normal starting material for the process will ordinarily be hot rolled and have a microstructure of equiaxed ferrite and pearlite. The cold reduction step deforms pearlite colonies and ferrite grains in a manner corresponding to the change in the dimensions of the material as a whole. Thus, both pearlite colonies and ferrite grains are elongated in the direction of principal deformation. The greater the amount of cold reduction, the longer and thinner the pearlite colonies and ferrite grains become. To achieve the desired elongation of the pearlite colonies, cold reduction of greater than 50% is required. This amount of reduction may, of course, be produced in any convenient manner, usually for example, by a number of deformation steps such as a plurality of passes through a rolling mill. The process in accordance with the invention does not require a segregated or so-called "banded" condition in the steel initially.

On reheating to the  $T_x$  temperature which is somewhat above the  $Ac_1$ , the elongated pearlite converts to austenite. Austenite forms almost exclusively in the pearlite and hence assumes a corresponding size, shape and distribution. The result is that just prior to quenching, the steel contains austenite particles which are long and thin, and all oriented alike, and having substantially the same chemical composition as the pearlite. Control of the reheat temperature  $T_x$ , is necessary to insure that austenite particles of this nature are present. If the reheat temperature is too low, pearlite is not fully converted to austenite. If too high, austenite grows into the ferrite and consequently is reduced in carbon content and becomes less fibrous. Also, in reheating, the cold worked ferrite matrix recrystallizes into annealed equiaxed grains. Because the reheat temperature is relatively low and the heating time short, a desirable fine grain size is developed in the ferrite.

Quenching to room temperature transforms the austenite fibers into martensite fibers. The hardenability of the austenite fibers is much greater than that of the fully austenitized steel because the fibers have substantially the composition of pearlite and hence contain close to the eutectoid carbon content. Moreover, because of the affinity of carbon for manganese, this element is also present to a greater extent in the fibers than in the steel as a whole. These features make it possible to apply the process to steels which contain substantially lower carbon and alloy contents than is otherwise required for quenching to all martensite structures.

The product produced by the process described herein contains a microstructure which comprises martensite fibers containing up to about 0.8% carbon imbedded in a fine-grained ferrite matrix. The fibers are, therefore, about 10 times as strong as the matrix. This microstructure, therefore, is a desirable composite material since the

strong martensite fibers tend to strengthen the more ductile ferrite matrix. Careful control of the reheat temperature, pointed out above, is essential to achieve this condition.

Subsequent processing may be performed to modify properties. Ductility is increased at some sacrifice in strength by tempering, e.g., at about 400° F. Higher strength and better machinability may be obtained by cold working as necessary, e.g. to up to about a 20% reduction in cross section.

It is within the purview of the invention to treat hypoeutectoid steels and in particular those preferably containing less than 0.35% carbon. However, carbon as well as low-alloy steels can be processed by the invention, although mechanical properties after processing will, of course, vary with the type of steel. The following is provided as further examples of the process as described herein.

A 1-inch diameter hot-rolled bar of AISI 1015 steel containing 0.16% carbon and 0.51% manganese was cold swaged to 0.25-inch diameter. It was then reheated by immersing in a lead bath at 1380° F. for 2-minutes and then water quenched. This specimen is designated as Example A in Table I below. For comparison, an identical 0.25-inch diameter rod was normalized from 1700° F. and is included in Table I as Sample B. To illustrate further improvements obtainable, a specimen similar to Sample A was additionally tempered at 400° F. for 1-hour and is reported in Table I as Sample C to show how a different combination of yield strength and ductility may be obtained within the purview of the invention.

TABLE I

| Sample | Tensile strength (p.s.i.) | Yield strength (p.s.i.) | Red. of area (percent) | Elong. in 1-in. (percent) |
|--------|---------------------------|-------------------------|------------------------|---------------------------|
| A----- | 136,900                   | 69,100                  | 19                     | 12                        |
| B----- | 61,300                    | 43,000                  | 71                     | 35                        |
| C----- | 102,000                   | 61,500                  | 53                     | 21                        |

The examples described above in Table I demonstrate the strength that results in a low-carbon steel by processing in accordance with the invention.

Tensile properties of strip of several grades of steel processed according to the process hereof and all subsequently tempered at 400° F. for 2-hours are described in Table II. With each steel of the examples the starting material was 0.5-inch thick hot-rolled plate. The plates were cold rolled to 0.15-inch, reheated to  $T_x \pm 20^\circ$  F. and water quenched.

TABLE II

| AISI Grade       | C    | Mn   | Si    | Ni    | Cr    | Mo    | Tensile strength (p.s.i.) | Yield strength (p.s.i.) | Elong. in 1-in. (percent) |
|------------------|------|------|-------|-------|-------|-------|---------------------------|-------------------------|---------------------------|
| 1010-----        | 0.11 | 0.55 | ----- | ----- | ----- | ----- | 84,100                    | 55,800                  | 22.5                      |
| 1011 (Mod.)----- | .12  | 1.10 | .20   | ----- | ----- | ----- | 118,700                   | 79,600                  | 19                        |
| 1020-----        | .20  | .53  | .24   | ----- | ----- | ----- | 91,700                    | 68,700                  | 27                        |
| 1026-----        | .24  | .86  | .23   | ----- | ----- | ----- | 137,100                   | 78,200                  | 13.5                      |
| 1034-----        | .35  | .37  | .21   | ----- | ----- | ----- | 114,000                   | 78,500                  | 14                        |
| 1021+.5 Ni-----  | .21  | .79  | ----- | .49   | ----- | ----- | 133,000                   | 74,100                  | 15.5                      |
| 1320-----        | .21  | 2.00 | .27   | ----- | ----- | ----- | 159,900                   | 109,000                 | 17                        |
| 4310-----        | .12  | .81  | .28   | 1.75  | .77   | .22   | 124,500                   | 97,800                  | 21                        |
| 4320-----        | .21  | .73  | .25   | 1.80  | .80   | .21   | 195,700                   | 153,000                 | 11.5                      |

## References Cited

## UNITED STATES PATENTS

3,423,252 1/1969 Grange 148-12

L. DEWAYNE RUTLEDGE, Primary Examiner

W. W. STALLARD, Assistant Examiner

The strengths obtained in the various representative hypoeutectoid carbon and low-alloy steels in Table II are the result of processing to develop a fibrous martensite-ferrite microstructure. Tempering at 400° F. as the samples in Table II were, further improves the ductility and yield strength combination. If the tempering step is omitted, substantially higher tensile strengths may be obtained but with lower ductility. As indicated previously, additional strength and enhancement of machinability is imparted by cold working as necessary, e.g. up to about a 20% reduction in cross section.

The fibrous martensite-ferrite mixture is a type of microstructure which is not developed by conventional processing or heat treating, and the properties resulting therefrom include potentially useful characteristics such as unusually high rate of work hardening, relatively good machinability and resistance to certain kinds of corrosive attack.

In view of the foregoing, it is apparent that various changes and modifications may be made without departing from the invention. Accordingly, the scope of the invention should be limited only by the appended claims whereby what is claimed is:

1. A method of processing carbon and low-alloy steels to develop a fibrous martensite-ferrite mixture which comprises cold reducing an article of said steel to at least a 50% smaller cross sectional area than initially to elongate said article, heating said cold reduced article to a temperature in the range of  $(T_x) \pm 20^\circ$  F. where  $T_x$  is determined by the following equation:

$$T_x (\text{° F.}) = 1385 - (25 \times \% \text{ Mn}) + (40 \times \% \text{ Si}) - (26 \times \% \text{ Ni}) + (42 \times \% \text{ Cr})$$

and quenching to transform austenite fibers to martensite.

2. A method in accordance with claim 1 wherein the starting material is in the hot-rolled condition.

3. A method in accordance with claim 1 wherein the starting material is in the heat-treated condition.

4. A method in accordance with claim 1 wherein the product produced thereby is cold worked to enhance strength and improved machinability.

5. A method in accordance with claim 4 wherein said product is cold worked up to about 20%.

6. A method in accordance with claim 1 wherein, after quenching, said article is tempered to improve ductility.

7. A method in accordance with claim 6 wherein said tempering is at 400° F.

8. A method in accordance with claim 6 wherein, after tempering, the steel is cold worked to enhance strength and improve machinability.